

# United States Patent [19]

Becker et al.

[11] 3,721,555

[45] March 20, 1973

[54] **DIFFUSION TRANSFER RECEPTION  
ELEMENTS, FILM UNITS AND  
PROCESSES THEREFOR**

[75] Inventors: **Richard W. Becker; Glen M. Dap-  
pen**, both of Rochester, N.Y.

[73] Assignee: **Eastman Kodak Company**,  
Rochester, N.Y.

[22] Filed: **Aug. 24, 1971**

[21] Appl. No.: **174,505**

[52] U.S. Cl. .... **96/29 D, 96/3, 96/76 C,  
96/77, 96/84 R**

[51] Int. Cl. .... **G03c 7/00, G03c 5/54, G03c 1/40**

[58] Field of Search ..... **96/3, 29 D, 84 R**

[56] **References Cited**

**UNITED STATES PATENTS**

3,635,707 1/1972 Cole ..... 96/3

*Primary Examiner—J. Travis Brown  
Assistant Examiner—Alfonso Suro Pico  
Attorney—Robert W. Hampton et al.*

[57] **ABSTRACT**

Vinyl polymers containing anionic solubilizing groups are employed as the binder in a light-reflective layer which is associated with a dye image-receiving layer employed in color diffusion transfer systems.

**22 Claims, No Drawings**

**DIFFUSION TRANSFER RECEPTION ELEMENTS,  
FILM UNITS AND PROCESSES THEREFOR**

This invention relates to the art of photography and more particularly to color diffusion transfer film units, 5 reception elements and methods for obtaining stable, positive, right-reading diffusion transfer dye images of high quality.

U.S. Pat. No. 3,227,550 of Whitmore and Mader is-  
sued Jan. 4, 1966 and U.S. Pat. No. 3,227,552 of Whit-  
more issued Jan. 4, 1966 describe photographic image  
transfer processes wherein an immobile coupler is  
reacted with oxidized color developer to form a mobile  
dye which is transferred by diffusion to a receiving  
layer to form a color image. During the development 15  
phase of the color development diffusion transfer  
process, the image dyes formed in the respective blue,  
green and red-sensitive silver halide emulsion layers  
diffuse into an image-receiving layer of the receiving  
element where the dyes are mordanted to form the  
transferred image. At the same time, small amounts of  
development reaction products and unused color  
developer diffuse into the image-receiving layer. When  
the receiving element is separated from the photosensi- 20  
tive element, oxygen in the atmosphere causes rapid  
oxidation of the unused developer, self-coupling of the  
developer occurs, thereby producing a yellowish-  
brown stain, particularly in the highlight or minimum  
density areas. 25

U.S. Pat. No. 3,445,228 issued May 20, 1969 of 30  
Beavers et al. discloses that a white pigment contained  
in an interlayer of a dye image-receiving element for  
use in the above-described process conceals the stain  
formed in an acid layer and functions also as a timing  
layer. Specific binders mentioned include gelatin, 35  
polyvinyl alcohol and other vinyl polymers. It would be  
desirable to provide an image-receiving element  
wherein higher maximum dye densities are obtainable  
both initially and after incubation.

Accordingly, it is an object of this invention to pro-  
vide a film unit employing an image-receiving element  
capable of receiving stable dye images of high quality  
and process of using same.

It is another object of this invention to provide an  
image-receiving element providing higher maximum  
dye densities of the transferred image, both initially and  
after subjecting to various atmospheric conditions for  
extended periods of time.

It is another object of this invention to provide a film  
unit employing an image-receiving element having an  
increased rate of dye diffusion transfer in comparison  
to the prior art.

These and other objects are achieved by a photo-  
graphic film unit according to our invention, which is  
adapted to be processed by passing the unit between a  
pair of juxtaposed pressure-applying members, such as  
would be found in a camera designed for in-camera  
processing, comprising:

- a. a photosensitive element comprising a support  
having thereon at least one, and preferably three,  
photosensitive silver halide emulsion layers, each  
silver halide emulsion layer having associated  
therewith a dye image-providing material;
- b. a dye image-receiving layer having a light-reflect-  
ing layer associated therewith comprising a vinyl  
polymer containing anionic solubilizing groups  
and an opacifying agent; and

c. a rupturable container containing an alkaline  
processing composition and which is adapted to be  
positioned during processing of the film unit so  
that a compressive force applied to the container  
by pressure-applying members in a camera will ef-  
fect a discharge of the container's contents within  
the film unit.

Our invention can be used not only in diffusion  
transfer systems wherein the image-receiving element  
is located on a separate support from the photosensi- 10  
tive element, but also in diffusion transfer systems  
wherein the image-receiving element is integral with  
the photosensitive element.

In one embodiment of our invention wherein the  
image-receiving element is separate from the photosensi- 15  
tive element, the novel dye image-receiving element  
comprises a support having thereon the following  
layers:

- a. a light-reflecting layer comprising a vinyl polymer  
containing anionic solubilizing groups and an  
opacifying agent, and

- b. a dye image-receiving layer.

The above-described dye image-receiving element of  
the film unit is adapted to be superposed on the  
photosensitive element after exposure thereof. The  
development and transfer operations can be effected  
by bathing either or both the exposed photosensitive  
element and the dye image-receiving element in a  
developing solution before rolling into contact with  
each other, or a viscous developing composition can be  
placed between the elements for spreading in a  
predetermined amount across and into contact with the  
exposed surface of the photosensitive element. The  
viscous developing composition is desirably utilized in  
one or more pods attached to the reception sheet or  
photosensitive element that can be readily ruptured  
when development is desired as described, for example,  
in U.S. Pats. Nos. 2,559,643; 2,647,049; 2,661,293;  
2,698,244; 2,698,798 and 2,774,668.

During the development phase of a color diffusion  
transfer process according to our invention, the dye  
image-providing material formed in the respective  
blue-, green- and red-sensitive silver halide emulsion  
layers diffuse out of the photosensitive element through  
the viscous developer composition and into the dye  
image-receiving layer, e.g., into the dye image-receiving  
element described above, where the dyes are mordanted  
to form the transferred image.

In another embodiment of our invention, the dye  
image-receiving layer is located integral with the  
photosensitive element between the support and the  
lowermost photosensitive silver halide emulsion layer.  
Such integral receiver-negative photosensitive ele-  
ments are described in copending U.S. application Ser.  
No. 115,459 of Barr, Bush and Thomas filed Feb. 16,  
1971 and now abandoned. In such an embodiment, the  
support for the photosensitive element is transparent  
and is coated with the dye image-receiving layer, the  
light-reflective layer described above and the various  
layers forming the color-forming units. After exposure  
of the photosensitive element, a rupturable container  
containing an alkaline processing composition and an  
opaque process sheet are brought into superposed position.  
Pressure-applying members in a camera rupture  
the container and spread processing composition over  
the photosensitive element as the film unit is withdrawn

from the camera. The processing composition develops the exposed silver halide layers and dye images are formed as a function of development which diffuse to the image-receiving layer to provide a positive, right-reading image which is viewed through the transparent support on the opaque reflecting layer background. For further details concerning this particular film unit, its preparation and use, reference is made to the above-mentioned U.S. application Ser. No. 115,459 of Barr, Bush and Thomas filed Feb. 16, 1971.

Another embodiment of integral receiver-negative photosensitive systems in which our invention can be employed is described in U.S. Ser. No. 115,552 of Cole filed Feb. 16, 1971 and now abandoned. In such an embodiment, the support for the color diffusion transfer system is transparent and is coated with the image-receiving layer, the light-reflective layer described above and then the various layers forming the color-forming units and a top transparent sheet. A rupturable container containing an alkaline processing composition and an opacifier is positioned adjacent to the top layer and sheet. The film unit is placed in a camera, exposed through the top transparent sheet and then passed between a pair of pressure-applying members in the camera as it is being removed therefrom. The pressure-applying members rupture the container and spread processing composition and opacifier over the negative portion of the film unit to render it light-insensitive. The processing composition develops the exposed silver halide layers and dye images are formed as a result of development which diffuse to the image-receiving layer to provide a positive, right-reading image which is viewed through the transparent support on the opaque reflecting layer background. For further details concerning this particular integral film unit, its preparation and use, reference is made to the above-mentioned Cole U.S. application Ser. No. 115,552 filed Feb. 16, 1971.

Any vinyl polymer containing anionic solubilizing groups such as carboxyl groups or sulfonic acid groups can be employed in the light-reflecting layer according to our invention with good results. In certain embodiments highly preferred polymers are copolymers comprising recurring units of acrylic acid, sulfoalkyl acrylate or sulfoalkyl methacrylate with the remaining units of these copolymers derived from other ethylenically unsaturated monomers such as, for example, alkyl acrylates, alkyl methacrylates, etc. For further details concerning these polymers and their preparation, reference is made to U.S. Pat. No. 3,411,911 of Dykstra issued Nov. 19, 1968; U.S. Pat. No. 3,411,912 of Dykstra et al. issued Nov. 19, 1968; U.S. Pat. No. 3,488,708 of Smith issued Jan. 6, 1970; and U.S. Pat. No. 3,220,844 of Houck et al. issued Nov. 30, 1965. Examples of these preferred polymers include copoly(ethylacrylate, acrylic acid, 2-acetoacetoxyethyl methacrylate), copoly(ethylacrylate, acrylic acid) and copoly(n-butyl acrylate, 3-acryloxypropane-1-sulfonic acid sodium salt, 2-acetoacetoxy ethyl methacrylate).

The film assembly of our invention can be used to produce positive images in single or multicolors. In a three-color system, each silver halide emulsion layer of the film assembly of our invention will have associated therewith a dye image-providing material possessing a spectral absorption range substantially complementary

to the predominant sensitivity range of its associated emulsion, i.e., the blue-sensitive silver halide emulsion layer will have a yellow dye image-providing material associated therewith, the green-sensitive silver halide emulsion layer will have a magenta dye image-providing material associated therewith, and the red-sensitive silver halide emulsion layer will have a cyan dye image-providing material associated therewith. The dye image-providing material associated with each silver halide emulsion layer can be contained either in the silver halide emulsion layer itself or in a layer contiguous to the silver halide emulsion layer.

Spectral sensitizing dyes can be used conveniently to confer additional sensitivity to the light sensitive silver halide emulsion of the multilayer photographic elements of the invention. For instance, additional spectral sensitization can be obtained by treating the emulsion with a solution of a sensitizing dye in an organic solvent or the dye may be added in the form of a dispersion as described in Owens et al. British Pat. No. 1,154,781 issued June 11, 1969. For optimum results, the dye can either be added to the emulsion as a final step or at some earlier stage.

Sensitizing dyes useful in sensitizing such emulsions are described, for example, in Brooker et al., U.S. Pat. No. 2,526,632, issued Oct. 24, 1950; Sprague U.S. Pat. No. 2,503,776, issued Apr. 11, 1950; Brooker et al. U.S. Pat. No. 2,493,748, issued Jan. 10, 1950; and Taber et al., U.S. Pat. No. 3,384,486 issued May 21, 1968. Spectral sensitizers which can be used include the cyanines, merocyanines, complex (tri or tetrานuclear) merocyanines, complex (tri or tetrานuclear) cyanines, holopolar cyanines, styryls, hemicyanines (e.g., enamine hemicyanines), oxonols and hemioxonols. Dyes of the cyanine classes can contain such basic nuclei as the thiazolines, oxazolines, pyrrolines, pyridines, oxazoles, thiazoles, selenazoles and imidazoles. Such nuclei can contain alkyl, alkylene, hydroxyalkyl, sulfoalkyl, carboxyalkyl, aminoalkyl and enamine groups and can be fused to carbocyclic or heterocyclic ring systems either unsubstituted or substituted with halogen, phenyl, alkyl, haloalkyl, cyano, or alkoxy groups. The dyes can be symmetrical or unsymmetrical and can contain alkyl, phenyl, enamine or heterocyclic substituents on the methine or polymethine chain. The merocyanine dyes can contain the basic nuclei mentioned above as well as acid nuclei such as thiohydantoins, rhodanines, oxazolidenediones, thiazolidenediones, barbituric acids, thiazolineones, and malononitrile. These acid nuclei can be substituted with alkyl, alkylene, phenyl, carboxyalkyl, sulfoalkyl, hydroxyalkyl, alkoxyalkyl, alkylamino groups, or heterocyclic nuclei. Combinations of these dyes can be used, if desired. In addition, supersensitizing addenda which do not absorb visible light can be included, for instance, ascorbic acid derivatives, azaindenes, cadmium salts, and organic sulfonic acids as described in McFall et al. U.S. Pat. No. 2,933,390 issued Apr. 19, 1960 and Jones et al. U.S. Pat. No. 2,937,089 issued May 17, 1960.

The various silver halide emulsion layers of a color film assembly of the invention can be disposed in the usual order, i.e., the blue-sensitive silver halide emulsion layer first with respect to the exposure side, followed by the green-sensitive and red-sensitive silver ha-

lide emulsion layers. If desired, a yellow dye layer or a Carey Lea silver layer can be present between the blue-sensitive and green-sensitive silver halide emulsion layer for absorbing or filtering blue radiation that may be transmitted through the blue-sensitive layer. If desired, the selectively sensitized silver halide emulsion layers can be disposed in a different order, e.g., the blue-sensitive layer first with respect to the exposure side, followed by the red-sensitive and green-sensitive layers.

The silver halide emulsions used in this invention can comprise, for example, silver chloride, silver bromide, silver chlorobromide, silver bromoiodide, silver chlorobromoiodide or mixtures thereof. The emulsions can be coarse or fine grain and can be prepared by any of the well-known procedures, e.g., single jet emulsions such as those described in Trivelli and Smith, *The Photographic Journal*, Vol. LXXIX, May, 1939 (pp 330-338), double jet emulsions, such as Lippmann emulsions, ammoniacal emulsions, thiocyanate or thioether ripened emulsions such as those described in Nietz et al. U.S. Pat. No. 2,222,264 issued Nov. 19, 1940; Illingsworth U.S. Pat. No. 3,320,069 issued May 16, 1967; and McBride U.S. Pat. No. 3,271,157 issued Sept. 6, 1966. Surface image emulsions can be used or internal image emulsions can be used such as those described in Davey et al U.S. Pat. No. 2,592,250 issued May 8, 1952; Porter et al. U.S. Pat. No. 3,206,313 issued Sept. 14, 1965; Berriman U.S. Pat. No. 3,367,778 issued Feb. 6, 1968; and Bacon et al. U.S. Pat. No. 3,447,927 issued June 3, 1969. The emulsions may be regular grain emulsions such as the type described in Klein and Moisar, *J. Phot. Sci.*, Vol. 12, No. 5, Sept./Oct., 1964, (pp. 242-251). Negative type emulsions may be used or direct positive emulsions may be used such as those described in Leermakers U.S. Pat. No. 2,184,013 issued Dec. 19, 1939; Kendall et al. U.S. Pat. No. 2,541,472 issued Feb. 13, 1951; Berriman U.S. Pat. No. 3,367,778 issued Feb. 6, 1968; Schouwenaars British Pat. No. 723,019 issued Feb. 2, 1955; Illingsworth et al. French Pat. No. 1,520,821 issued Mar. 4, 1968; Illingsworth U.S. Pat. No. 3,501,307 issued Mar. 17, 1970; Ives U.S. Pat. No. 2,563,785 issued Aug. 7, 1951; Knott et al. U.S. Pat. No. 2,456,953 issued Dec. 21, 1948; and Land U.S. Pat. No. 2,861,885 issued Nov. 25, 1958.

The emulsions used with this invention may be sensitized with chemical sensitizers, such as with reducing agents; sulfur, selenium or tellurium compounds; gold, platinum or palladium compounds; or combinations of these. Suitable procedures are described in Sheppard et al. U.S. Pat. No. 1,623,499 issued Apr. 5, 1927; Waller et al. U.S. Pat. No. 2,399,083 issued Apr. 23, 1946; McVeigh U.S. Pat. No. 3,297,447 issued Jan. 10, 1967; and Dunn U.S. Pat. No. 3,297,446 issued Jan. 10, 1967.

The silver halide emulsions used with this invention may contain speed increasing compounds such as polyalkylene glycols, cationic surface active agents and thioethers or combinations of these as described in Piper U.S. Pat. No. 2,886,437 issued May 12, 1959; Dann et al. U.S. Pat. No. 3,046,134 issued July 24, 1962; Carroll et al. U.S. Pat. No. 2,944,900 issued July 12, 1960; and Goffe U.S. Pat. No. 3,294,540 issued Dec. 27, 1966.

The silver halide emulsions used in the practice of this invention can be protected against the production of fog and can be stabilized against loss of sensitivity during keeping. Suitable antifoggants and stabilizers each used alone or in combination include thiazolium salts described in Brooker et al. U.S. Pat. No. 2,131,038 issued Sept. 27, 1938; and Allen et al. U.S. Pat. No. 2,694,716 issued Nov. 16, 1954; the azaindenes described in Piper U.S. Pat. No. 2,886,437 issued May 12, 1959; and Heimbach et al. U.S. Pat. No. 2,444,605 issued July 6, 1948; the mercury salts as described in Allen et al. U.S. Pat. No. 2,728,663 issued Dec. 27, 1955; the urazoles described in Anderson et al U.S. Pat. No. 3,287,135 issued Nov. 22, 1966; the sulfocatechols described in Kennard et al. U.S. Pat. No. 3,236,652 issued Feb. 22, 1966; the oximes described in Carroll et al. British Pat. No. 623,448 issued May 18, 1949; nitrogen; nitroindazoles; the mercaptotetrazoles described in Kendall et al. U.S. Pat. No. 2,403,927 issued July 16, 1946; Kennard et al. U.S. Pat. No. 3,266,897 issued Aug. 16, 1966; and Luckey et al. U.S. Pat. No. 3,397,987 issued Aug. 20, 1968; the polyvalent metal salts described in Jones U.S. Pat. No. 2,839,405 issued June 17, 1958; the thiuronium salts described in Herz et al. U.S. Pat. No. 3,220,839 issued Nov. 30, 1965; the palladium, platinum and gold salts described in Trivelli et al. U.S. Pat. No. 2,566,263 issued Aug. 28, 1951; and Yutzy et al U.S. Pat. No. 2,597,915 issued May 27, 1952; and the tetrazoles described in Hoppe U.S. Pat. No. 3,352,672 issued Nov. 14, 1967.

Any dye image-providing material can be employed in this invention as long as an imagewise distribution of the material will be formed after development as a function of the imagewise exposure of the silver halide emulsion to which the dye image-providing material is associated. For example, there may be employed as the dye image-providing material dye developers as illustrated by U.S. Pat. No. 2,983,606; coupling dyes as disclosed, for example, in U.S. Pat. No. 3,087,817; "shifted" or "leuco" dye developers; dye developer precursors; metal dye complexes as disclosed, for example, in U.S. Pats. Nos. 3,185,567 and 3,453,107; couplers requiring an oxidizing agent in the image-receiving layer to form a color; "ring-closing" dye developers as disclosed in U.S. Pat. No. 3,443,943; color-providing materials as disclosed in U.S. Pats. Nos. 3,443,940 and 3,443,941; etc.

Particularly good results are obtained in this invention when the dye image-providing material associated with each silver halide emulsion layer is a nondiffusible coupler which produces a diffusible dye upon reaction with oxidized aromatic primary amino color developing agents, such as p-phenylenediamine developing agents. Such couplers include those having the formulas:

DYE - LINK - (COUP - BALL)<sub>n</sub>

and

BALL - LINK - (COUP - SOL)<sub>n</sub>

wherein

- 60 1. DYE is a dye radical exhibiting selective absorption in the visible spectrum and containing an acidic solubilizing radical;

2. LINK is a connecting radical such as an azo radical, a mercuri radical, an oxy radical, an alkylidene radical, a thio radical, a dithio radical or an azoxy radical;
3. COUP is a coupler radical such as a 5-pyrazolone coupler radical, a pyrazolotriazole coupler radical, a phenolic coupler radical or an open-chain ketomethylene coupler radical, COUP being substituted in the coupling position with LINK;
4. BALL is a photographically inert organic ballasting radical of such molecular size and configuration as to render such coupler nondiffusible during development in the alkaline processing composition;
5. SOL is a hydrogen atom or an acidic solubilizing group when the color developing agent contains an acidic solubilizing group, and SOL is an acidic solubilizing group when the color developing agent is free of an acidic solubilizing group; and
6.  $n$  is an integer of 1 to 2 when LINK is an alkylidene radical, and  $n$  is 1 when LINK is an azo radical, a mercuri radical, an oxy radical, a thio radical, a dithio radical or an azoxy radical.

For further details concerning the above-described couplers, their preparation and use, reference is made to U.S. Pat. No. 3,227,550 of Whitmore et al. issued Jan. 4, 1966; U.S. Pat. No. 3,227,552 of Whitmore issued Jan. 4, 1966; and British Pat. No. 904,364, page 19, lines 1-41.

If the silver halide emulsion employed with the non-diffusible couplers described above is a direct positive silver halide emulsion, such as an internal image emulsion or a solarizing emulsion, which is developable in unexposed areas, a positive image can be obtained on the dye image-receiving layer. In this embodiment, the nondiffusible coupler can be located in the silver halide emulsion itself. After exposure of the film unit, the alkaline processing composition permeates the various layers to initiate development of the exposed photosensitive silver halide emulsion layers. The aromatic primary amino color developing agent present in the film unit develops each of the silver halide emulsion layers in the unexposed areas (since the silver halide emulsions are direct positive ones), thus causing the developing agent to become oxidized imagewise corresponding to the unexposed areas of the direct positive silver halide emulsion layers. The oxidized developing agent then reacts with the nondiffusible coupler present in each silver halide emulsion layer to form imagewise distributions, respectively, of diffusible cyan, magenta and yellow dye as a function of the imagewise exposure of each of the silver halide emulsion layers. At least a portion of the imagewise distributions of diffusible cyan, magenta and yellow dye diffuse to the image-receiving layer to provide a positive dye image upon separation of the receiver from the negative.

Internal image silver halide emulsions useful in the above-described embodiment are direct positive emulsions that form latent images predominantly inside the silver halide grains, as distinguished from silver halide grains that form latent images predominantly on the surface thereof. Such internal image emulsions were described by Davey et al. in U.S. Pat. No. 2,592,250 issued Apr. 8, 1952, and elsewhere in the literature.

These emulsions can also contain fogging or nucleating agents such as those described in U.S. Pats. Nos. 2,588,982; 2,563,785; 3,227,552; etc.

As previously mentioned, the aromatic primary amino color developing agent employed in the above-described embodiment is preferably present in the alkaline processing composition in the rupturable pod. The color developing agent can also be incorporated into the negative portion of the film unit as a separate layer, e.g., by employing a Schiff base derivative of an aromatic primary amino color developing agent such as that formed by reacting o-sulfobenzaldehyde and N,N-diethyl-3-methyl-4-aminoaniline. Such incorporated developing agent will be activated by the alkaline processing composition. While the incorporated developing agent can be positioned in any layer of the photosensitive element from which it can be readily made available for development upon activation with alkaline processing composition, it is generally either incorporated in the light-sensitive silver halide emulsion layers or in layers contiguous thereto. As mentioned above, aromatic primary amino color developing agents employed in certain embodiments of this invention are preferably p-phenylenediamine developing agents. These developing agents are well known to those skilled in the art and include the following compounds and salts thereof: 4-amino-N,N-diethyl-3-methyl aniline, N,N-diethyl-p-phenylenediamine, N-ethyl- $\beta$ -methane-sulfonamido-ethyl-3-methyl-4-aminoaniline, 4-amino-N-ethyl-3-methyl-N- $\beta$ -sulfoethyl)aniline, 4-amino-N-ethyl-3-methoxy-N-( $\beta$ -sulfoethyl)aniline, 4-amino-N-ethyl-N-( $\beta$ -hydroxyethyl)aniline, 4-amino-N,N-diethyl-3-hydroxymethyl aniline, 4-amino-N-methyl-N-( $\beta$ -carboxyethyl)aniline, 4-amino-N,N-bis-( $\beta$ -hydroxyethyl)aniline, 4-amino-N,N-bis( $\beta$ -hydroxyethyl)-3-methyl aniline, 3-acetamido-4-amino-N,N-bis( $\beta$ -hydroxyethyl)-aniline, 4-amino-N-ethyl-N-(2,3-dihydroxypropyl)-3-methyl aniline, 4-amino-N,N-diethyl-3-(3-hydroxypropoxy)aniline, and the like.

In a color film unit according to the invention, each silver halide emulsion layer containing a dye image-providing material or having the dye image-providing material present in a contiguous layer may be separated from the other silver halide emulsion layers in the negative portion of the film unit by materials in addition to those described above, including gelatin, calcium alginate, or any of those disclosed in U.S. Pat. No. 3,384,483, polymeric materials such as polyvinylamides as disclosed in U.S. Pat. No. 3,421,892, or any of those disclosed in U.S. Pats. Nos. 2,992,104; 3,043,692; 3,044,873; 3,061,428; 3,069,263; 3,069,264; 3,121,011; and 3,427,158.

Generally speaking, except where noted otherwise, the silver halide emulsion layers in the invention comprise photosensitive silver halide dispersed in gelatin and are about 0.6 to 6 microns in thickness; the dye image-providing materials are dispersed in an aqueous alkaline solution-permeable polymeric binder, such as gelatin, as a separate layer about 1 to 7 microns in thickness; and the alkaline solution-permeable polymeric interlayers, e.g., gelatin, are about 1 to 5 microns in thickness. Of course, these thicknesses are approximate only and can be modified according to the product desired. In addition to gelatin, other suitable

hydrophilic materials include both naturally-occurring substances such as proteins, cellulose derivatives, polysaccharides such as dextran, gum arabic and the like; and synthetic polymeric substances such as water soluble polyvinyl compounds like poly(vinylpyrrolidone), acrylamide polymers and the like.

The photographic emulsion layers and other layers of a photographic element employed in the practice of this invention can also contain alone or in combination with hydrophilic, water-permeable colloids, other synthetic polymeric compounds such as dispersed vinyl compounds such as in latex form and particularly those which increase the dimensionl stability of the photographic materials. Suitable synthetic polymers include those described, for example, in Nottorf U.S. Pat. No. 3,142,568, issued July 28, 1964; White U.S. Pat. No. 3,193,386, issued July 6, 1965; Houck et al. U.S. Pat. No. 3,062,674, issued Nov. 6, 1962; Houck et al. U.S. Pat. No. 3,220,844, issued Nov. 30, 1965; Ream et al. U.S. Pat. No. 3,287,289, issued Nov. 22, 1966; and Dykstra U.S. Pat. No. 3,411,911, issued Nov. 19, 1968. Particularly effective are water-insoluble polymers of alkyl acrylates and methacrylates, acrylic acid, sulfoalkyl acrylates or methacrylates, those which have cross-linking sites which facilitate hardening or curing described in Smith U.S. Pat. No. 3,488,708 issued Jan. 6, 1970, and those having recurring sulfobetaine units as described in Dykstra Canadian Pat. No. 774,054.

Any material can be employed as the image-receiving layer in this invention as long as the desired function of mordanting or otherwise fixing the dye images will be obtained. The particular material chosen will, of course, depend upon the dye to be mordanted. If acid dyes are to be mordanted, the image-receiving layer can contain basic polymeric mordants such as polymers of amino guanidine derivatives of vinyl methyl ketone such as described in Minsk U.S. Pat. No. 2,882,156 issued Apr. 14, 1959, and basic polymeric mordants such as described in copending U.S. Application Ser. No. 100,491 of Cohen et al. filed Dec. 21, 1970 and now abandoned. Other mordants useful in our invention include poly4-vinylpyridine, the 2-vinyl pyridine polymer metho-p-toluene sulfonate and similar compounds described in Sprague et al. U.S. Pat. No. 2,484,430 issued Oct. 11, 1949, and cetyl trimethylammonium bromide, etc. Effective mordanting compositions are also described in Whitmore U.S. Pat. No. 3,271,148 and Bush U.S. Pat. No. 3,271,147, both issued Sept. 6, 1966.

Furthermore, the image-receiving layer can be sufficient by itself to mordant the dye as in the case of use of an alkaline solution-permeable polymeric layer such as N-methoxy methyl polyhexylmethylen adipamide; partially hydrolyzed polyvinyl acetate; polyvinyl alcohol with or without plasticizers; cellulose acetate; gelatin; and other materials of a similar nature. Generally, good results are obtained when the imagereceiving layer, preferably alkaline solution-permeable, is transparent and about 0.25 to about 0.04 mil in thickness. This thickness, of course, can be modified depending upon the result desired. The image-receiving layer can also contain ultra-violet absorbing materials to protect the mordanted dye images from fading due to ultraviolet light, brightening agents such as the stilbenes, coumarins, triazines, oxazoles,

dye stabilizers such as the chromanols, alkylphenols, etc.

Use of a pH-lowering material associated with the dye image-receiving element of the invention will usually increase the stability of the transferred image. Generally, the pH-lowering material will effect a reduction in the pH of the image layer from about 13 or 14 to at least 11 and preferably 5-8 within a short time after imbibition. For example, polymeric acids as disclosed in U.S. Pat. No. 3,362,819; or metallic salts, e.g., zinc acetate, zinc sulfate, magnesium acetate, the formates, acetates, propionates, stearates, nitrates, or sulfates of zinc, aluminum, iron, manganese, cobalt of nickel, etc.; or solid acids as disclosed in U.S. Pat. No. 2,584,030 may be employed with good results. Such pH-lowering materials reduce the pH of the film unit after development to terminate development and substantially reduce further dye transfer and thus stabilize the dye image. The pH-lowering material can be present as a separate layer between the light-reflecting layer and its support where the image-receiving element is separate from the photosensitive element or can be located between the light-reflecting layer and the lowermost silver halide emulsion layer in an integral receiver-negative element.

Any opacifying agent can be employed in the light-reflecting layer according to our invention. Particularly desirable are white opacifying agents since they would provide an esthetically pleasing background on which to view a transferred dye image and would possess the optical properties desired for reflection of incident radiation. Suitable opacifying agents include: titanium dioxide, barium sulfate, zinc oxide, barium stearate, silver flake, silicates, alumina, zirconium oxide, zirconium acetyl acetate, sodium zirconium sulfate, kaolin, mica, or mixtures thereof in widely varying amounts depending upon the degree of opacity desired. Especially good results are obtained with titanium dioxide. Zinc oxide in combination with titanium dioxide may also be employed to great advantage as disclosed and claimed in copending application Ser. No. 174,443 of Abbott, Dappen and Irani filed of even date herewith. Brightening agents such as the stilbenes, coumarins, triazines and oxazoles can also be added to the opacifying layer if desired. It is believed that any stain resulting from excess developing agent or oxidized developing agent is hidden or masked by this layer.

Where a pH-lowering layer is employed, such as a polymeric acid layer, the vinyl polymer containing anionic solubilizing groups in the opacifying layer will function as a "timing" layer and will control the pH reduction of the dye image-receiving element as a function of the rate at which the alkali diffuses through the layer. Of course, widely varying amounts of the vinyl polymer containing anionic solubilizing groups can be employed in the opacifying layer, depending upon the results desired.

The alkaline processing composition employed in this invention is the conventional aqueous solution of an alkaline material, e.g., sodium hydroxide, sodium carbonate or an amine such as diethylamine, preferably possessing a pH in excess of 12. The solution also preferably contains a viscosity-increasing compound such as a high molecular weight polymer, e.g., a water-soluble ether inert to alkaline solutions such as hydrox-

ethyl cellulose or alkali metal salts of carboxymethyl cellulose such as sodium carboxymethyl cellulose. A concentration of viscosity-increasing compound of about 1 to about 5 percent by weight of the processing solution is preferred which will impart thereto a viscosity of about 100 cps. to about 200,000 cps.

While the alkaline processing composition used in this invention can be employed in a rupturable container, as described previously, other methods of applying processing composition could also be employed, e.g., bathing the photosensitive element in a processing bath, interjecting processing composition with communicating members similar to hypodermic syringes which are attached either to a camera or camera cartridge, etc.

While the film units of our invention can be modified so as to be employed in roll form, they are preferably used in cartridges similar to those described in U.S. Pat. Nos. 3,080,805; 3,161,118; and 3,161,122; said patents also illustrating typical cameras for performing color diffusion transfer processes of our invention.

The supports for the photographic elements of this invention can be any material as long as it does not deleteriously effect the photographic properties of the film unit and is dimensionally stable. Typical materials include cellulose nitrate film, cellulose acetate film, poly(vinyl acetal) film, polystyrene film, poly(ethyleneterephthalate) film, polycarbonate film, poly- $\alpha$ -olefins such as polyethylene and polypropylene film, and related films or resinous materials as well as glass, paper, metal, etc. The support is usually about 2 to 6 mils in thickness.

While the invention has been described with reference to layers of silver halide emulsions and dye image-providing materials, dotwise coating, such as would be obtained using a gravure printing technique, could also be employed. In this technique, small dots of blue, green and red-sensitive emulsions have associated therewith, respectively, dots of yellow, magenta and cyan color-providing substances. After development, the transferred dyes would tend to fuse together into a continuous tone.

The photographic layers employed in the practice of this invention may contain surfactants such as saponin; anionic compounds such as the alkyl aryl sulfonates described in Baldsiefen U.S. Pat. No. 2,600,831 issued June 17, 1952; amphoteric compounds such as those described in Ben-Ezra U.S. Pat. No. 3,133,816 issued May 19, 1964; and water soluble adducts of glycidol and an alkyl phenol such as those described in Olin Mathieson British Pat. No. 1,022,878 issued Mar. 16, 1966; and Knox U.S. Pat. No. 3,514,293 issued May 26, 1970.

The various layers, including the photographic layers, employed in the practice of this invention can contain light absorbing materials and filter dyes such as those described in Sawdey U.S. Pat. No. 3,253,921 issued May 31, 1966; Gaspar U.S. Pat. No. 2,274,782 issued Mar. 3, 1942; Silberstein et al. U.S. Pat. No. 2,527,583 issued Oct. 31, 1950; and VanCampen U.S. Pat. No. 2,956,879 issued Oct. 18, 1960.

The sensitizing dyes and other addenda used in the practice of this invention can be added from water solutions or suitable organic solvent solutions may be used. The compounds can be added during various

procedures including those described in Collins et al. U.S. Pat. No. 2,912,343 issued Nov. 10, 1959; McCrossen et al. U.S. Pat. No. 3,342,605 issued Sept. 19, 1967; Audran U.S. Pat. No. 2,996,287 issued Aug. 15, 1961 and Johnson et al. U.S. Pat. No. 3,425,835 issued Feb. 4, 1969.

The photographic layers used in the practice of this invention may be coated by various coating procedures including dip coating, air knife coating, curtain coating, or extrusion coating using hoppers of the type described in Beguin U.S. Pat. No. 2,681,294 issued June 15, 1954. If desired, two or more layers may be coated simultaneously by the procedures described in Russell U.S. Pat. No. 2,761,791 issued Sept. 4, 1956; Hughes U.S. Pat. No. 3,508,947 issued Apr. 28, 1970; and Wynn British Pat. No. 837,095 issued June 9, 1960. This invention also can be used for silver halide layers coated by vacuum evaporation as described in British Pat. No. 968,453 issued Sept. 2, 1964 and Lu-Valle et al. U.S. Pat. No. 3,219,451 issued Nov. 23, 1965.

The photographic and other hardenable layers used in the practice of this invention can be hardened by various organic or inorganic hardeners, alone or in combination, such as the aldehydes, and blocked aldehydes as described in Allen et al. U.S. Pat. No. 3,232,764 issued Feb. 1, 1966; ketones, carboxylic and carbonic acid derivatives, sulfonate esters, sulfonyl halides and vinyl sulfonyl ethers as described in Burness et al. U.S. Pat. No. 3,539,644 issued Nov. 10, 1970; active halogen compounds, epoxy compounds, aziridines, active olefins, isocyanates, carbodiimides, polymeric hardeners such as oxidized polysaccharides like dialdehyde starch and oxyguargum and the like.

The following examples further illustrate the invention.

#### EXAMPLE 1

40 Dye image-receiving elements are prepared by coating the following layers in the order recited on a transparent cellulose acetate film support:

1. Mordant layer of methyl-tri-n-dodecylammonium p-toluenesulfonate (22 mg/ft<sup>2</sup>), N-n-hexadecyl-n-morpholinium ethosulfate (150 mg/ft<sup>2</sup>) and gelatin (650 mg/ft<sup>2</sup>),
2. Interlayer of gelatin (100 mg/ft<sup>2</sup>), and
3. Light-reflecting layer of titanium dioxide (3000 mg/ft<sup>2</sup>) and the compounds identified in Table I below (300 mg/ft<sup>2</sup>)

50 A photographic element is prepared by coating the following layers in the order recited on a transparent support:

1. Gelatin (454 mg/ft<sup>2</sup>),
2. Gelatin-silver bromoiodide emulsion (300 mg of gelatin/ft<sup>2</sup> and 100 mg. of silver/ft<sup>2</sup>) and magenta dye image transfer coupler 1-phenyl-3-(3,5-disulfonylbenzamido)-4-(6-hydroxy-4-pentadecylphenylazo)-5-pyrazolone, dipotassium salt (75 mg/ft<sup>2</sup>), and
3. Overcoat of gelatin (100 mg/ft<sup>2</sup>)

55 Samples of the above photosensitive element are flash exposed. The following processing composition is spread from a pod between the exposed surface of the elements and the superposed image-receiving elements by passing the transfer "sandwich" between a pair of juxtaposed pressure rollers:

|                                                                         |         |
|-------------------------------------------------------------------------|---------|
| 4-amino-3-methoxy-N-ethyl-N- $\beta$ -hydroxyethylanilino hydrochloride | 30 g.   |
| sodium thiosulfate                                                      | 6 g.    |
| piperidino hexose reductone                                             | 0.8 g.  |
| hydroxyethyl cellulose                                                  | 32.0 g. |
| sodium hydroxide                                                        | 30.0 g. |
| water to                                                                | 1 liter |

The dye diffusion transfer time in seconds is observed for the first appearance of magenta dye in the dye image-receiving layer. After 60 seconds at about 20°C., the dye image-receiving element is peeled apart from the negative and the green reflection densities for both fresh and incubated coatings are measured. The following results are obtained:

TABLE I

| Polymer in Light-Reflecting Layer                                                               | First appearance of dye (sec.) | ΔD max. Fresh 1 wk. at D max. 49°C/50%RH | ΔD max. 5 wks. at 20°C/50%RH |
|-------------------------------------------------------------------------------------------------|--------------------------------|------------------------------------------|------------------------------|
| Gelatin (control)                                                                               | 14                             | 1.24                                     | -0.11                        |
| Poly(vinyl alcohol) (control)                                                                   | 11                             | 1.48                                     | -0.10                        |
| Copoly(ethylacrylate, acrylic acid, 2-acetoacetoxyethyl methacrylate) (71.8:23.8:4.4 by weight) | 10                             | 1.35                                     | -0.01                        |
| Copoly(ethylacrylate, acrylic acid) (80:20 by weight)                                           | 10                             | 1.31                                     | -0.05                        |

The above results indicate the higher Dmax. which can be obtained in accordance with our invention in comparison with one of the materials of the prior art along with the enhanced keeping stability and the increased rate of dye diffusion transfer in comparison with both materials of the prior art.

## EXAMPLE 2

Dye image-receiving elements are prepared similar to those of Example 1 except that layer 3 contains titanium dioxide (2,500 mg/ft<sup>2</sup>) and the compounds identified in Table II below (125 mg/ft<sup>2</sup>). These dye image-receiving elements are then tested in accordance with the procedure described in Example 1 to give the following results:

TABLE II

| Polymer in Light-Reflecting Layer                                                                                                 | First appearance of dye (sec.) | fresh dmax. |
|-----------------------------------------------------------------------------------------------------------------------------------|--------------------------------|-------------|
| Gelatin                                                                                                                           | 40                             | 1.04        |
| Copoly(n-butyl acrylate, 3-acryloxy-propane-1-sulfonic acid sodium salt, 2-acetoacetoxyethyl methacrylate) (90.2:5.8:4 by weight) | 18                             | 1.65        |
| Copoly(ethylacrylate, acrylic acid, 2-acetoacetoxyethyl methacrylate) (71.8:23.8:4.4 by weight)                                   | 14                             | 2.00        |

The above results again indicate the higher Dmax. and increased rate of dye diffusion transfer which can be obtained in accordance with our invention in comparison with a prior art material.

The invention has been described in detail with particular reference to preferred embodiments thereof, but, it will be understood that variations and modifica-

tions can be effected within the spirit and scope of the invention.

We Claim:

1. In a photographic film unit which is adapted to be processed by passing said unit between a pair of juxtaposed pressure-applying members comprising:

- a photosensitive element comprising a support having thereon at least one photosensitive silver halide emulsion layer, each said silver halide emulsion layer having associated therewith a dye image-providing material;
- a dye image-receiving layer having a light-reflecting layer associated therewith; and
- a rupturable container containing an alkaline processing composition and which is adapted to be positioned during processing of said film unit so that a compressive force applied to said container by said pressure-applying members will effect a discharge of the container's contents within said film unit;

the improvement comprising employing as said light-reflecting layer a vinyl polymer containing anionic solubilizing groups and an opacifying agent.

2. The photographic film unit of claim 1 wherein said photosensitive element comprises a support having thereon a red-sensitive silver halide emulsion layer having associated therewith a cyan dye image-providing material comprising a nondiffusible coupler capable of reacting with oxidized aromatic primary amino color developing agent to produce a diffusible cyan dye, a green-sensitive silver halide emulsion layer having associated therewith a magenta dye image-providing material comprising a nondiffusible coupler capable of reacting with oxidized aromatic primary amino color developing agent to produce a diffusible magenta dye, and a blue-sensitive silver halide emulsion layer having associated therewith a yellow dye image-providing material comprising a nondiffusible coupler capable of reacting with oxidized aromatic primary amino color developing agent to produce a diffusible yellow dye; said film unit containing an aromatic primary amino color developing agent.

3. The film unit of claim 1 wherein said dye image-receiving layer is located in said photosensitive element between said support and the lowermost photosensitive silver halide emulsion layer, and said light-reflecting layer is located in said photosensitive element between said dye image-receiving layer and said lowermost photosensitive silver halide emulsion layer.

4. The film unit of claim 1 wherein said dye image-receiving layer is coated on a separate support and is adapted to be superposed on said photosensitive element after exposure thereof, and said light-reflecting layer is located between said dye image-receiving layer and its said support.

5. The film unit of claim 4 wherein said rupturable container is so positioned during processing of said film unit that a compressive force applied to said container by said pressure-applying members will effect a discharge of the container's contents between said dye image-receiving layer and the outermost layer of said photosensitive element.

6. The film unit of claim 1 which also contains a pH-lowering material.

7. The film unit of claim 1 wherein said opacifying agent is titanium dioxide.

8. The film unit of claim 1 wherein said vinyl polymer is a copolymer comprising units of acrylic acid, sulfoalkyl acrylate or sulfoalkyl methacrylate.

9. The film unit of claim 1 wherein said vinyl polymer is copoly(ethylacrylate, acrylic acid, 2-acetoacetoxyethyl methacrylate), copoly(ethylacrylate, acrylic acid) or copoly(n-butyl acrylate, 3-acryloxypropane-1-sulfonic acid sodium salt, 2-acetoacetoxy ethyl methacrylate). 5

10. In a photographic film unit which is adapted to be 10 processed by passing said unit between a pair of juxtaposed pressure-applying members comprising:

I. a photosensitive element comprising a support having thereon the following layers in sequence:

- a. a direct-positive, red-sensitive silver halide emulsion layer containing a nondiffusible coupler capable of reacting with oxidized aromatic primary amino color developing agent to produce a diffusible cyan dye; 15
- b. an alkaline solution-permeable interlayer containing a compound capable of scavenging oxidized aromatic primary amino color developing agent; 20
- c. a direct-positive, green-sensitive silver halide emulsion layer containing a nondiffusible coupler capable of reacting with oxidized aromatic primary amino color developing agent to produce a diffusible magenta dye; 25
- d. an alkaline solution-permeable interlayer containing a compound capable of scavenging oxidized aromatic primary amino color developing agent; and
- e. a direct-positive, blue-sensitive silver halide emulsion layer containing a non-diffusible coupler capable of reacting with oxidized aromatic primary amino color developing agent to produce a diffusible yellow dye; 30

each said nondiffusible coupler having the formula:

DYE - LINK - (COUP - BALL)<sub>n</sub>

or

BALL - LINK - (COUP - SOL)<sub>n</sub>

wherein:

1. DYE is a dye radical exhibiting selective absorption in the visible spectrum and containing an acidic solubilizing group;

2. LINK is a connecting radical selected from the group consisting of an azo radical, a mercuri radical, an oxy radical, an alkylidene radical, a thio radical, a dithio radical and an azoxy radical;

3. COUP is a coupler radical selected from the group consisting of a 5-pyrazolone coupler radical, a pyrazolotriazole coupler radical, a phenolic coupler radical and an open-chain ketomethylene coupler radical, said COUP being substituted in the coupling position with said LINK;

4. BALL is a photographically inert organic ballasting radical of such molecular size and configuration as to render said coupler nondiffusible during development in said alkaline processing composition;

5. SOL is selected from the group consisting of a hydrogen atom and an acidic solubilizing group

when said color developing agent contains an acidic solubilizing group, and SOL is an acidic solubilizing when said color developing agent is free of an acidic solubilizing group; and

6. n is an integer of 1 to 2 when said LINK is an alkylidene radical, and n is 1 when said LINK is a radical selected from the group consisting of an azo radical, a mercuri radical, an oxy radical, a thio radical, a dithio radical and an azoxy radical;

II. a dye image-receiving element comprising a support having thereon a dye image-receiving layer, said element being adapted to be superposed over said blue-sensitive silver halide emulsion layer after exposure of said photosensitive element; and

III. a rupturable container containing an alkaline processing composition and which is adapted to be positioned during processing of said film unit so that a compressive force applied to said container by said pressure-applying members will effect a discharge of the container's contents between said dye image-receiving layer and said blue-sensitive silver halide emulsion layer of said photosensitive element;

said film unit containing an aromatic primary amino color developing agent; the improvement comprising employing as said dye image-receiving element a support having thereon a polymeric acidic material layer, a light-reflecting layer, comprising a vinyl polymer containing anionic solubilizing groups and an opacifying agent, and a dye image-receiving layer.

11. The photographic film unit of claim 10 wherein said vinyl polymer is a copolymer comprising units of acrylic acid, sulfoalkyl acrylate or sulfoalkyl methacrylate and said opacifying agent is titanium dioxide.

12. The photographic film unit of claim 11 wherein said vinyl polymer is copoly(ethylacrylate, acrylic acid, 2-acetoacetoxyethyl methacrylate), copoly(ethylacrylate, acrylic acid) or copoly(n-butyl acrylate, 3-acryloxypropane-1-sulfonic acid sodium salt, 2-acetoacetoxy ethyl methacrylate).

13. A reception element comprising a support having thereon

- a. a light-reflecting layer comprising a vinyl polymer containing anionic solubilizing groups and an opacifying agent, and
- b. a dye image-receiving layer.

14. The reception element of claim 13 which includes a pH-lowering layer between said support and said layer a.

15. The reception element of claim 13 wherein said opacifying agent is titanium dioxide.

16. The reception element of claim 13 wherein said vinyl polymer is a copolymer comprising units of acrylic acid, sulfoalkyl acrylate or sulfoalkyl methacrylate.

17. The reception element of claim 16 wherein said vinyl polymer is copoly(ethylacrylate, acrylic acid, 2-acetoacetoxyethyl methacrylate), copoly(ethylacrylate, acrylic acid) or copoly(n-butyl acrylate, 3-acryloxypropane-1-sulfonic acid sodium salt, 2-acetoacetoxy ethyl methacrylate).

18. The reception element of claim 17 wherein said opacifying agent is titanium dioxide.

19. In a process of forming a transfer image comprising:

- a. imagewise-exposing a photosensitive element comprising a support having thereon at least one photosensitive silver halide emulsion layer, each said silver halide emulsion layer having associated therewith a dye image-providing material;
  - b. treating the layer outermost from the support of said exposed photosensitive element with an alkaline processing composition to effect development of each of said exposed silver halide emulsion layers;
  - c. forming an imagewise distribution of diffusible dye image-providing material as a function of said imagewise exposure of each said silver halide emulsion layer; and
  - d. at least a portion of each said imagewise distribution of diffusible dye image-providing material diffusing to a dye image-receiving layer having a light-reflecting layer associated therewith;
- the improvement comprising employing as said light-reflecting layer a vinyl polymer containing anionic solubilizing groups and an opacifying agent.

20. The process of claim 19 wherein said treatment step b. is effected by

- A. superposing over the layer outermost from the

5

10

15

20

25

30

35

40

45

50

55

60

65

support of said photosensitive element said dye image-receiving layer coated on a support, said light-reflecting layer being located between said dye image-receiving layer and its said support;

B. positioning a rupturable container containing said alkaline processing composition between said exposed photosensitive element and said dye image-receiving layer; and

C. applying a compressive force to said container to effect a discharge of the container's contents between said outermost layer of said exposed photosensitive element and said dye image-receiving layer.

21. The process of claim 20 wherein said vinyl polymer is a copolymer comprising units of acrylic acid, sulfoalkyl acrylate or sulfoalkyl methacrylate.

22. The process of claim 21 wherein said vinyl polymer is copoly(ethylacrylate, acrylic acid, 2-acetoacetoxyethyl methacrylate), copoly(ethylacrylate, acrylic acid) or copoly(n-butyl acrylate, 3-acryloxypropane-1-sulfonic acid sodium salt, 2-acetoacetoxy ethyl methacrylate).

\* \* \* \* \*